

Aug. 27, 1974

B. E. BARTON ET AL

3,832,295

FUSED SALT ELECTROLYSIS TO OBTAIN MANGANESE METAL

Filed Nov. 27, 1972



**INVENTORS**

PAUL H. CARDWELL  
BRUCE E. BARTON

# United States Patent Office

3,832,295

Patented Aug. 27, 1974

1

3,832,295

## FUSED SALT ELECTROLYSIS TO OBTAIN MANGANESE METAL

Bruce E. Barton, Houston, Tex., and Paul H. Cardwell,  
Zanoni, Va., assignors to Deepsea Ventures, Inc.

Filed Nov. 27, 1972, Ser. No. 309,624

Int. Cl. C22d 3/02, 3/18

U.S. Cl. 204—64 R

12 Claims

### ABSTRACT OF THE DISCLOSURE

This invention provides a method for obtaining molten manganese metal by electrolyzing a molten mixture of metal halides comprising a manganese halide and a bath mixture comprising a halide of a reactant metal, an alkali metal halide and an alkaline earth metal halide. Manganese metal is obtained in a molten phase below the molten mixture of metal halides and elemental halogen is evolved at the anode. The reactant metal is electrolytically reduced at the cathode. The anode and cathode are both inert and immersed in the molten mixture of metal halides.

The halides are preferably chlorides, bromides or iodides. The reactant metal can be any cathodically reducible metal which can replace manganese from manganese halide in the molten salt bath, but is preferably aluminum or magnesium.

Many non-ferrous metals are commercially produced at relatively low cost; however, although the metal is suitable for certain purposes, it is too impure for other possible uses. It thus often becomes necessary to go to substantial additional expense to purify the metal, which was obtained, for example, by reduction of compounds found in the ores. Manganese, for example, has some uses which are satisfied by a relatively low grade purity metal, e.g., in which the manganese can contain carbon silicon or iron. For other purposes, however, an extremely high purity material is required in which the presence of any carbon, silicon, or iron would be detrimental. For other uses, only certain of the impurities impose a problem and the presence of other impurities is not detrimental. For example, manganese is often found in iron or steel products. For such uses the presence of even a relatively small percentage of carbon would be deleterious as is could have a significant effect upon the properties of the steel in which the manganese is present. The presence of a small proportion of iron in the manganese would have substantially little or no effect on the final properties of such a product.

Another factor is the form of the metal obtained from the process. For example, there is often a requirement that the metal be in special form, e.g., in large chunks or ingots.

Manganese, for example, has been prepared by several methods; generally, all of these methods comprise reducing a manganese oxide to the elemental metal. Such reduction has been carried out by displacing the manganese from the oxide using aluminum metal, by reducing using carbon, or by electrolysis such as in a fused salt bath. The reduction of the manganese oxide by contact at high temperatures with carbon or aluminum does result in a relatively large size chunk of the metal, but unfortunately, it does not result in a high purity product.

The electrolysis of oxides of manganese in a fused salt bath has been carried out and this does result in large chunks or ingots of metal of relatively good purity, if great care is taken. The procedures wherein manganese oxide is reduced have been extremely expensive, however.

Various fused salt electrolysis methods have been carried out, wherein the manganese feed has been manganese oxide ores, mixtures of ferro-manganese and calcium fluoride and calcium manganite. These, however, were generally unsuccessful in preparing high purity manganese metal products.

2

An early worker in the field, Mitchell, in U.S. Pat. No. 2,398,589, suggested the electrolysis of manganese oxides in a fused bath containing an alkali metal fluoride plus an aluminum or magnesium oxide. For example, the bath comprised sodium fluoride, aluminum oxide or magnesium oxide, and a manganese oxide, preferably MnO. In order to avoid the problem of additional impurities being dissolved from the container material, the sides of the cell were lined with manganese oxide. Manganese metal was formed as a solid mass on the bottom of the cell. A metal cathode was located at the bottom of the cell and a carbon anode was located at the top of the cell. The current flow was in a vertical direction.

The problem of removing a solid mass of manganese from the bottom of the fused bath cell was difficult and subsequent workers, such as Welsh et al., in work described in U.S. Pat. No. 3,018,233, devised methods to obtain molten manganese metal which could then be removed by tapping the cell at regular intervals. Welsh et al. disclosed that an oxide of boron, aluminum or silicon can be added to the manganese oxide-calcium fluoride salt to increase the solubility of the manganese oxide in the electrolyte. The boron oxide, for example, is added in almost equal proportions with the manganese oxide. Welsh et al. formed a molten layer of manganese at the bottom of the cell which then acted as the cathode. A carbon anode was used projecting downwardly from the top of the cell. The current flow was in a vertical direction through the fused salt mass.

Although Welsh et al. was an improvement over Mitchell, the same problem arose with regard to the presence of oxides which generally make it substantially impossible to avoid at least some contamination of the metal by the high melting, high boiling oxide materials.

It has now been discovered that it is possible in accordance with the present invention to obtain substantial pure molten manganese in a cell utilizing inert anodes and cathodes in which the molten electrolyte is comprised only of halides. The product from the cell of this invention is a pure manganese metal in which the presence of oxides is substantially eliminated and from which substantially all of the reaction products formed during the electrolysis are removed by vaporization, resulting in the production of manganese metal which is substantially pure.

In accordance with the present invention, a process for forming substantially pure molten manganese metal is provided. The process comprises first forming a molten mixture of halides, comprising a manganese halide, a bath halide selected from the group consisting of alkali metal halides and alkaline earth metals halides, and a halide of a reactant metal. The reactant metal can be any cathodically reducible metal which can replace manganese from its halide, but is preferably magnesium or aluminum.

The mixed fused halide bath is electrolyzed to form manganese metal which sinks through the bath and collects as a molten layer at the bottom of the bath while halogen is collected at the anode. Heat is applied to the bottom of the bath to maintain the manganese metal in a molten state while the top of the bath is preferably maintained at a sufficiently low temperature to prevent the vaporization and loss of metal halides, but at least about 650° C. A temperature gradient can be maintained through the molten bath to avoid vaporization of any halides.

The apparatus in which the electrolysis procedure is carried out is a furnace wherein the upper portion of the furnace is a fused salt electrolytic cell and the lower portion is a molten metal collection section. The temperature maintained in the lower metal collection portion of the furnace is sufficient to maintain the manganese metal in

the molten condition, but the temperature in the upper cell portion of the furnace is sufficient to maintain the metal halides in a molten condition, but is below the boiling point of the metal halide mixture. The electrodes are located in the upper, or cell portion, of the furnace and the flow of electricity is in a horizontal direction across the bath.

It is believed that the present process does not result in the direct cathodic reduction of the manganese halide to manganese metal. Rather, it is believed that the halide of the reactant metal, e.g., magnesium halide or aluminum halide, is cathodically reduced to form the halogen and the reactant metal. The, e.g., magnesium metal or aluminum metal which is formed then reacts with the manganese halide present in the bath, replacing the manganese in the halide salt to form elemental manganese metal and the e.g. aluminum halide or magnesium halide. The elemental manganese metal then sinks to the bottom of the halide bath to form a layer of molten manganese metal.

The potential drop between the electrodes is not sufficient to cathodically reduce the manganese halide to manganese metal. It is believed that the potential drop is sufficient, under the conditions of the process of this invention, to cathodically reduce the halide of the reactant metal to the elemental reactant metal.

Preferably, the temperature of the halide bath is above the melting point of the reactant metal, e.g. 650° C. for magnesium and 660° C. for aluminum.

Preferably, the reactant metal is formed as small particles or droplets dispersed in the molten mixed metal halide bath. This provides a greater surface area for reaction between the reactant metal and the manganese halide. To further prevent the agglomeration of the molten reactant metal, an anti-agglomerating agent is added, which serves to maintain the molten reactant metal in a dispersed state in the molten halide bath. This is especially useful when magnesium halide is present.

The bath halide and the halide of the reactant metal are miscible with manganese halide but immiscible with manganese metal. The bath halides are generally inert to the manganese halide under the conditions of this process and do not react with the cathodically reduced reactant metal, e.g. magnesium or aluminum. They are essentially inert with regard to manganese metal and generally, are non-corrosive to the usual types of high temperature ceramic liners available.

The bath halides must be a mixture of at least one alkali metal halide and at least one alkaline earth metal halide. The mixture can form a low melting eutectic composition so as to reduce the temperature, at least in the upper electrolysis cell portion of the apparatus.

Certain of the halides used, especially manganese halides and aluminum halides (if used as reactant halides) have relatively high vapor pressures under the conditions of the electrolysis cell. Aluminum halides, in the pure state, boil at temperatures substantially lower than those under which these cells are normally operated, e.g. about 650° C. and higher. However, when the aluminum halides are admixed with the alkali and/or alkaline earth metal halides of the bath halide, the vapor pressure of the mixture is substantially reduced, apparently by the formation of certain complexes, and the boiling point of the mixture at atmospheric pressure is raised to substantially above 650° C.

Preferably, there is present at least one alkali metal halide. Useful alkali metal halides comprise the chlorides, iodides, and bromides of sodium, potassium, cesium, rubidium and lithium. Useful alkaline earth metal halides comprise the chlorides, bromides, and iodides of calcium, barium, strontium, and magnesium.

In determining composition of the molten halide mixture, the "bath mixture," refers to the combined "reactant halide" and "bath halide," i.e. everything except the manganese halides.

The bath mixture comprises from about 30 to about 60% by wt. of the bath mixture of an alkali metal halide, about 10 to about 25% by wt. of a halide of a reactant metal and from about 15 to about 60% by wt. of an alkaline earth metal halide. It is understood by the above stated ranges of composition, that when, e.g. a magnesium halide is utilized as the halide of a reactant metal, the total proportion of magnesium halide present in the bath mixture can be from about 10 to about 70% by wt. of the bath mixture.

In addition, there is preferably also present in the bath mixture a small proportion of an anti-agglomerating agent, such as an alkali metal tetraborate; generally, not more than 0.05% by wt. of the compound and preferably from 0.001 to about 0.01% by wt.

There can be present from about 0.2 to about 90% by wt. of the total mixture of a manganese halide. Preferably, however, the manganese halide is present in an amount of from about 0.5 to about 30% by wt., and optimally from 0.5 to about 10% by wt.

The temperature of the salt bath should be just sufficient to maintain the halide and preferably also the reactant metal in the molten condition. It is desirable to avoid loss by vaporization of any of the volatile halides. This is especially true of the aluminum halide if used.

Accordingly, the temperature of the top surface of the molten mixed halide bath can vary from 650° C. up to about 1260° C. When aluminum halide is used as the reactant halide, at higher temperatures, the volatile halide can be lost by vaporization. Accordingly, the preferred temperature for the top surface of the mixed halide bath containing aluminum halide is from about 650° C. to about 1,000° C. and preferably about 800° C. to about 1,000° C. The molten manganese layer at the bottom of the bath is preferably maintained in the range of from about 1,260° C. to about 1,300° C.

Useful anti-agglomerating agents includes boric oxide or metal salts or boric acids for example  $B_2O_3$ ,  $Na_2B_4O_7$  and  $K_2B_2O_4$ .

The drawing is a vertical section of a proposed combination fused salt electrolytic cell furnace.

Referring to the drawing, the fused salt electrolytic cell furnace includes an insulating brick outer shell 10, a refractory brick lid 12, and a high temperature-resistant inert liner 32, such as high purity alumina in brick or solid sheet form, or high purity zirconia in brick or solid sheet form. The liner is supported by a metal backing 34; graphite anodes, 24 and 28, extend through the top of lid 12 into the cell and are connected, via conductors 20 and 21, to the anode bus of an electrical power source, not shown. A steel cathode, 26, extends into the cell and is connected, via electrical conductors 22, to the cathode bus of an electrical power source, not shown. Solid feed inlet ports 16 and 17, are provided extending through the refractory lid 12, and vapor outlet ports 14 and 18 are also provided through refractory lid 12.

The lower portion of the furnace is formed as a relatively narrow neck 38 from which a liquid outlet port 40 is provided. The lower narrow portion 38 is coaxial with the larger portion 42 of the furnace and is surrounded by heating chamber 36. A bleed line 23 is provided from the upper portion 42 of the furnace.

Heating elements are positioned within the heating chamber 36. Any conventional heating elements can be provided in chamber 36. Molten manganese is recovered through tap 40.

The anodes 24 and 28 are preferably formed of graphite. The cathode 26 is preferably formed of steel. The electrodes must be inert to the fused salt medium, the halogen and the manganese metal and reactant metal. The cathode must be formed of a material having a sufficiently high melting point that it is not softened or weakened during the electrolysis when immersed in the fused molten salt bath.

The outlet port for the molten metal and the bleed line for the molten metal halides are conventional in the art. Basically, such ports include an outlet which can be stopped by a removable clog of refractory material. The molten material can be removed continuously or intermittently as desired in a continuous process. Designs of such outlets are well known in the art. See, for example, U.S. Pats. Nos. 3,018,233 and 2,309,598.

Any heat source can be used in chamber 36. Gas jets and electrical coils are useful, or alternatively, heating coils can be positioned within the reactor vessel portion, 38, or heating electrode plates can be provided flush within the walls 32, of the lower portion, 38.

In operation, it is extremely important to prevent the presence of oxygen or any oxides in the bath, except for the antiagglomeration agent. Metal oxides tend to increase the amount of impurities in the manganese metal. Accordingly, before adding any manganese halide to the cell, the cell is preferably flushed with an inert oxygen-free gas, such as nitrogen or any other inert material, to remove all air, after the bath halides have been added to the cell and heated to a temperature sufficient to melt all of the halides including the alkali metal, alkaline earth metal halides and any other reactant metal halide present. The lower portion of the melt in the narrow neck portion 38 is preferably maintained at a temperature of at least about 1260° C. and can be kept as high as 1300° C.

When the temperature of the bath has been set, the electrodes are energized to the desired voltage dependent upon the reactant metal used. Manganese halide is added through solid inlet ports, 16, and 17. The manganese halide melts as it mixes with the fused salt bath.

Halogen is evolved at the anodes and can be withdrawn through ports 14 and 18.

Gradually, a layer of molten manganese metal is collected in the narrow neck portion 38. This molten manganese metal can be intermittently removed through tap 40.

Generally, the manganese halide that is added to the cell will not be completely pure. Manganese halide which is obtained, for example, from the refining of ocean floor nodule ore, such as for example, is described in German Patent Specification No. 2,126,175 contains substantial proportions of sodium halide, magnesium halide, potassium halide, lithium halide, and calcium halide. Thus, the bath is being fed not only with the manganese halide, which is being reduced and removed, but also additional alkali and alkaline earth metal halides. In order to prevent a buildup of the halides in the cell and to maintain a substantially constant cell bath concentration, a continuous or intermittent bleed is maintained through exit port 23 from the electrolysis cell. The rate of bleed through line 23 must be balanced against the rate of feed of the impure manganese halide and the composition of the feed material in order to maintain a substantially constant electrolyte concentration.

As stated above, it is believed that the present procedure does not result in the direct electrolysis of manganese. The electrolysis occurs as the cathodic reduction of the reactant halide, e.g. magnesium halide or aluminum halide, to form e.g. magnesium metal or aluminum metal and the elemental halogen. The halogen is removed at the anode. Under the conditions of the cell, all of the halogens, i.e., chlorine, iodine or bromine are in the vaporous state and can be readily removed. The reactant metal, e.g. aluminum or magnesium which is formed remains in the salt bath and reacts with the manganese halide, displacing the manganese to reform magnesium halide or aluminum halide and the elemental manganese metal. The elemental manganese metal sinks through the molten halide bath to collect as a lower layer in the narrow neck, or furnace, portion 38, of the cell-furnace combination. Thus, there is substantially no net loss of the reactant halide, e.g., magnesium halide or aluminum halide, from the cell.

The manganese halide must be replaced in the bath during electrolysis. The rate at which the manganese halide is consumed is dependent upon the rate at which the reactant metal is formed, which in turn is dependent upon the current flow. The rate of feed of the manganese halide must be sufficient to maintain a sufficient concentration of manganese halide in the electrolysis bath to react with the reactant metal to form manganese metal and the halide of the reactant metal.

10 The following examples provide preferred embodiments of the present invention, but are exemplary and not exclusive of the scope thereof:

#### EXAMPLE 1

15 A sample of mixed metal chlorides was prepared having the following composition by weight:

| Components:        | Percent by Weight |
|--------------------|-------------------|
| Sodium Chloride    | 59.8              |
| Magnesium Chloride | 24.9              |
| Calcium Chloride   | 15.0              |
| Sodium Tetraborate | 0.3               |

20 A 10,000 gram sample of the above mixture was added to an alumina-lined electrolyte cell, of the type shown in the drawing, and melted to form a fused molten salt bath.

25 The temperature in the lower portion 38 of the furnace in the drawing, was 1260° C. The temperature of the upper surface of the bath was 840° C.

30 The electrodes were energized and a potential drop of 6.4 volts was formed between the electrodes at a current density of 500 amps/sq. ft. After 15 minutes of operation, anhydrous manganese chloride 58 grams was added. The test was continued until 300 ampere-hours of current had passed and a total of 580 grams of anhydrous manganese chloride had been added. The voltage drop between the electrodes had decreased from 6.4 to 5.0 during this period and the temperature of the upper portion of the bath had increased to 895° C.

35 Manganese metal was produced during the test and collected in the lower narrow portion 38 of the cell. The metal was periodically tapped and removed through port 40.

40 The current efficiency of the electrolysis based upon the amount of manganese collected was 80 percent. Chlorine was evolved and removed through the ports 14 and 18.

#### EXAMPLE 2

45 A mixture of metal halides having the following composition is prepared

| Components:       | Percent by Weight |
|-------------------|-------------------|
| Sodium Chloride   | 40                |
| Aluminum Chloride | 20                |
| Calcium Chloride  | 40                |

50 A sample of 10,000 grams of the above salt mixture is melted as described in Example 1 in the combined electrolysis cell furnace, shown in the drawing. The temperature of the upper portion of the melt is maintained at 860° C. The temperature at the very bottom portion 38 is 60 maintained at 1260° C. The electrodes are energized and a potential drop of 6.3 volts and a current density of 500 amp/sq. ft. is applied between the electrodes. After the current has been applied for 15 minutes, 58 grams of anhydrous manganese chloride is added to the bath. The test is continued until a total of 300 ampere hours of current has been passed and 580 grams of manganese chloride has been added to the electrolysis cell.

65 Manganese metal was collected in the bottom portion 38 of the cell furnace. Manganese metal was intermittently tapped and removed through tap 40.

70 The patentable embodiments of this invention which are claimed are as follows:

1. A process for the forming of substantially pure molten manganese metal from manganese halide, the process comprising: (1) forming a molten mixture of

metal halides, the halides being selected from the group consisting of chlorides, bromides and iodides, the molten mixture comprising a manganese halide and a bath mixture comprising a halide of a reactant metal, an alkali metal halide and an alkaline earth metal halide; (2) passing an electric current through said molten mixture between an inert anode and an inert cathode immersed within the molten mixture of halides; (3) electrolytically reducing the reactant metal at the cathode; (4) evolving at and collecting from the anode an elemental halogen, and collecting molten manganese metal below the molten mixture of halides.

2. The process of Claim 1 wherein the reactant metal is selected from the group consisting of aluminum and magnesium.

3. The process of Claim 2 wherein the temperature of the lower portion of the bath immediately adjacent to the manganese metal is maintained at least at the melting point of manganese metal, and the temperature of the upper portion of the bath is maintained at least at the melting point of the mixed halides.

4. The process of Claim 2 wherein the reactant metal is aluminum.

5. The process of Claim 2 wherein the composition of the bath mixture comprises from about 30 to about 60 percent by weight of an alkali metal halide, from about 10 to about 25 percent by weight of a halide of a reactant metal and from about 15 to about 60 percent by weight of an alkaline earth metal halide.

6. The process of Claim 2 wherein the reactant metal is magnesium.

7. The process of Claim 3 wherein the temperature of the top portion of the molten metal halide bath is at least about 660° C.

8. The process of Claim 2 wherein the halide is chloride and the halogen is chlorine.

9. The process of Claim 5 wherein the bath mixture comprises sodium chloride, calcium chloride, and magnesium chloride.

10. The process of Claim 2 wherein the concentration of manganese halide in the molten mixture of halides is in the range of from about 0.5 to about 10% by wt.

11. The process of Claim 5, wherein the bath mixture comprises in addition an anti-agglomerating agent.

12. A process in accordance with Claim 11, wherein the anti-agglomerating agent is selected from the group consisting of boric oxide, boric acids and alkali metal salts thereof.

#### References Cited

#### UNITED STATES PATENTS

3,450,524 6/1969 Pascaud et al. \_\_\_\_\_ 204—64 R  
3,535,215 10/1970 Winand \_\_\_\_\_ 204—64 R

JOHN H. MACK, Primary Examiner

D. R. VALENTINE, Assistant Examiner

U.S. Cl. X.R.

204—245